

## UNITED STATES PATENT OFFICE

2,202,364

## LUBRICATING OIL

Peter J. Wiezevich, now by judicial change of name to Peter J. Gaylor, Elizabeth, N. J., assignor to Standard Oil Development Company, a corporation of Delaware

No Drawing. Application April 3, 1937,  
Serial No. 134,838

## 4 Claims. (Cl. 87-9)

This invention relates to lubricating oils for use in internal combustion engines, and is more particularly concerned with improved addition agents therefor.

It is known that small quantities, that is, between 0.1 and 2%, of metallic soaps such as aluminum stearate, improve the properties of lubricating oils particularly with respect to lowering the pour point, decreasing the tendency to cause sludge deposits in the engine, and increasing oiliness. There is a serious objection to the use of these soaps, namely, that they do not remain dispersed in the oil but tend to settle out or cause gel formation on standing. This objection can be overcome to some extent by adding to the oil certain "solubilizing agents" which have the effect of retaining the metallic soaps in more or less complete dispersion in the oil.

It has now been found that metallic soaps, if prepared from certain acids, will remain completely dispersed in lubricating oils, such as wax-free lubricating fractions of petroleum, without the necessity of using a solubilizing agent and without sacrificing in any way the valuable properties imparted to the oil by the ordinary soaps such as aluminum stearate. The present invention is directed to these improved soaps and will be fully understood from the following description.

According to the present invention the metallic soaps are prepared from crude acids derived from the oxidation of paraffin wax, petrolatum or other waxy hydrocarbons. These crude acids may be obtained in the following manner: Paraffin wax is oxidized with air or other gas containing free oxygen at a substantially low temperature of between 200 and 350° F. for a period of 2 to 4 hours, preferably in an aluminum tower. Various catalytic materials such as potassium permanganate, manganese stearate or soda ash may be used as catalysts to promote the oxidation. The reaction product is then saponified with caustic soda preferably containing some methyl alcohol. Thereafter the mixture is thoroughly agitated and the aqueous layer is separated from the waxy layer. The wax and unsaponifiable compounds may be recovered from the latter by extraction with naphtha and then recycled to the oxidation. The aqueous layer containing the soaps and methyl alcohol is distilled to remove the alcohol, and sulfuric acid is then added to liberate the acids from the soaps. The liberated acids are washed and distilled and the product so obtained is the crude acid de-

sired. For the purposes of the present invention, the C<sub>10</sub> to C<sub>20</sub> fraction is preferred. The distillation is continued to about 480° F. under a 29 inch vacuum and the acids so obtained have an acid number of about 190 and a saponification number of about 240. Either the crude acids, or their fractions may be employed.

It has been found that it is desirable to employ acids substantially free of high molecular weight acids, say those above C<sub>20</sub> or C<sub>24</sub>, since the soaps of the latter do tend to settle out from oil.

From these crude acids metallic soaps are prepared. Aluminum is the preferred metal. Chromium, tin and manganese may also be used but they are not as effective as aluminum. Since the acids obtained by the oxidation of wax are generally considered to be similar chemically to fatty acids, it would be expected that the aluminum soaps would behave in the same manner as aluminum stearate. But this is not the case, especially with the crude acids obtained by the method disclosed above.

Since it does not take very much soap to cause a gel-like formation in oil, it is essential for the purpose of this invention to remove any traces of gel-forming compounds by dissolving the aluminum soaps of the crude acid or its fractions in naphtha or similar suitable solvent, and filtering out the small amount of insoluble soap which is present and which otherwise would cause gel formation in a lubricating oil.

When the metallic soaps of the crude acids are added to lubricating oils in amounts from 0.5 to about 5%, there results an improved lubricating oil of increased oiliness, and decreased sludging tendency. The latter property is especially observed when such blends are employed for the lubrication of Diesel engines. Apparently, the combustion characteristics of Diesel engines are considerably different from those encountered in the usual spark ignition automobile engines so that ordinary lubricants deteriorate much more rapidly and form a peculiar type of coating on the pistons. The soap prepared according to the invention remains completely dispersed in the oil and shows no tendency to separate out or gel on standing.

There is an indication that the presence of lactones or lactone-like materials are desirable in maintaining a non-stringy consistency in mineral oils. Hence, it is desirable, during saponification of the wax acids, to avoid excess alkali and thereby to prevent hydrolysis of such lactones or lactides. The best procedure is to make the

- acids neutral to litmus with alkali, and then some free wax acids are added to make certain that free alkalinity does not exist. It is also possible to add additional lactones or lactides to the wax acids prior to saponification or conversion to aluminum or other soap.

It will be understood that other agents may also be added to these oils, not for the purpose of solubilizing the soap, for this is not necessary, but rather to improve the oil with respect to other properties. Thus other oiliness agents, pour inhibitors, V. I. improvers, extreme pressure agents, volatized products, corrosion inhibitors, and sludge preventors may also be added as well as other agents such as oxidation inhibitors, thickeners, dyes, etc. The addition of corrosion inhibitors such as soluble peroxides or sulfur compounds such as phenol sulfides or polysulfides is especially useful. The effective compounds in the latter category are phenol sulfides having the formula:



where R may be H, or an alkyl radical, R' an alkyl, alkyl-aryl, or aryl radical, and n is an integer from 1 to 4.

30 The use of these improved soaps is not restricted to any particular type of lubricating oil but is applicable generally to all lubricating oil fractions whether obtained by the distillation, cracking, hydrogenation or other treatment of petroleum, coals, tars, lignites or fractions thereof. However, as pointed out above, the greatest value for such compositions is in the Diesel lubrication field.

It will be understood that wherever the term "crude acids" is used in the specification or appended claims, it means the product of oxidation of paraffin wax or other waxy hydrocarbons after removal of unoxidized wax but before the removal of any other constituents. Some of the non-saponifiable material may be removed, but it is desirable to allow a portion or all of it to remain in the crude acid mixture.

The following examples illustrate the application of the invention:

50

*Example I.*

200 grams of crude acid derived from the products of oxidation of wax and having the following characteristics

55 Acid number..... 205  
Molecular weight (calculated)..... 273  
Saponification number..... 238

are reacted with 56 grams of NaOH, an amount greater than that calculated to be necessary from 60 the acid number. Since it is preferable to avoid excess alkali, some additional wax acid is added until the mixture is neutral to litmus. The soap solution is placed in a separatory funnel and is slowly added to a relatively large quantity of hot water. The mass is agitated vigorously and simultaneously a concentrated solution of aluminum sulfate (100 grams of  $Al_2(SO_4)_3$ ) is added. The insoluble aluminum soap thereby formed is separated, and is washed first with aluminum 65 sulfate solution and then with water, followed by dissolving it in Varsol (heavy naphtha) and filtering. The soap contains 4.32% Al by analysis. It is dissolved in lubricating oil by heating for 3 hours at a temperature between 200 and 70 400° F.

1% of this aluminum soap is added to a lubricating oil. The following table shows the comparative inspections of the oil with and without the soap:

|                        | Oil alone | Oil+1% Al soap of crude acid | 5  |
|------------------------|-----------|------------------------------|----|
| Gravity, °A. P. I.     | 21.8      | 22.3                         |    |
| Flash, °F.             | 410       | 425                          | 10 |
| Fire, °F.              | 470       | 475                          |    |
| Saybolt vis. @ 100° F. | 726       | 771                          |    |
| Saybolt vis. @ 210° F. | 62.2      | 65                           |    |
| Pour point, °F.        | -5        | 0                            |    |
| Cloud point, °F.       | 123       | None                         |    |
| Color, Robinson        | 121       | 414                          |    |
| Colorhold              | 121       | 314                          | 15 |
| Carbon, Conradson      | 0.11      | 0.26                         |    |
| Neutralization number  | .04       | 1.94                         |    |
| Saponification number  |           | 2.60                         |    |

When the oil without any soap was run in a C. F. R. engine it had a demerit rating of 1.43. On the other hand, when the oil containing 1% of the Al soap was run in the same engine, it had a demerit rating of only 0.93.

*Example II*

25

In another experiment 1% of an Al soap of the crude acid containing only 2.92% Al was added to the same oil as used in Example I. The following table shows the comparative inspections:

|                        | Oil alone | Oil+1% Al soap of crude acid | 30 |
|------------------------|-----------|------------------------------|----|
| Gravity, °A. P. I.     | 21.8      | 21.8                         |    |
| Flash, °F.             | 410       | 425                          |    |
| Fire, °F.              | 470       | 475                          |    |
| Saybolt vis. @ 100° F. | 726       | 752                          |    |
| Saybolt vis. @ 210° F. | 62.2      | 68.4                         |    |
| Pour point, °F.        | -5        | -5                           |    |
| Cloud point, °F.       | 123       | None                         |    |
| Color, Robinson        | 121       | 414                          | 40 |
| Colorhold              | 121       | 314                          |    |
| Carbon, Conradson      | 0.11      | 0.13                         |    |
| Neutralization number  | .04       | 0.80                         |    |
| Saponification number  |           | 1.90                         |    |

When the oil without any soap was run in a C. F. R. engine it had a demerit rating of 1.43. The oil containing 1% of the Al soap had a demerit rating of only 1.30 under the same conditions.

The term "demerit rating" as used in the above examples is a value arrived at after inspection of the used oil and all of the engine parts in contact therewith. The value is such that the smaller the number, the better the performance.

In the runs using the oil containing 1% of the aluminum soap, no ring sticking occurred and the "varnish" formation was considerably less than with the unblended oils, especially in the case of the soap containing the greater amount of aluminum. The carbon formation was also considerably less with the blended oils than with the unblended.

This invention is not limited by any theories of the mechanism of the action of metallic soaps on lubricating oils nor by any details which have been given merely for purposes of illustration, but is limited only in and by the following claims in which it is intended to claim all novelty inherent in the invention.

I claim:

1. An improved motor oil comprising a substantially wax-free viscous mineral oil and a small percentage of a soluble non-gelling aluminum soap of acids derived from the product of mild oxidation of waxy hydrocarbons, said acids

70

75

80

85

90

95

100

having not over 24 carbon atoms, and possessing the property of increasing the oxidation rate of the mineral oil.

2. Composition according to claim 1 in which the aluminum soap is present in amounts between 0.5 and 5%.

3. An improved motor oil comprising a viscous wax-free mineral oil and a small percentage of an aluminum soap of crude acids in the C<sub>10</sub> to C<sub>20</sub> molecular weight range derived from the product of mild oxidation of paraffin wax said

soap having the property of increasing the oxidation rate of the mineral oil.

4. A substantially wax-free lubricating oil for Diesel engine lubrication containing 0.5 to 3% of Al soaps of crude acids obtained by low temperature oxidation of petroleum wax, substantially free of acids of over 24 carbon atoms and possessing the property of increasing the oxidation rate of the mineral oil.

10

PETER J. WIEZEVICH.